

May 22, 1923.

1,456,035

M. H. NEWELL

METAL DUST AND PROCESS OF MAKING THE SAME

Filed Sept. 23, 1918



WITNESS

J. B. Gardner

INVENTOR

M. H. NEWELL

BY white & Post

HIS ATTORNEYS

## UNITED STATES PATENT OFFICE.

MINTON H. NEWELL, OF SAN FRANCISCO, CALIFORNIA, ASSIGNOR TO THE ALLOYS COMPANY, OF SAN FRANCISCO, CALIFORNIA, A CORPORATION OF CALIFORNIA.

## METAL DUST AND PROCESS OF MAKING THE SAME.

Application filed September 23, 1918. Serial No. 255,314.

To all whom it may concern:

Be it known that I, MINTON H. NEWELL, a citizen of the United States, and a resident of the city and county of San Francisco and State of California, have invented a certain new and useful Metal Dust and Process of Making the Same, of which the following is a specification.

The invention relates to a process for manufacturing metal dust and an improved product obtained by the practice of the process.

The object of the invention is to provide a better process for manufacturing metal dust and a better product. The invention is of particular value in the manufacture of zinc dust.

Zinc dust is largely used in a number of arts, but the characteristics measuring its efficiency have not been fully understood.

An object of this invention is to produce a zinc dust in very fine particles generally uniform in size and spherical in shape. Heretofore zinc dust has been comparatively inefficient because known processes of manufacture have resulted in products which comprised particles too large in size or particles vary in size and shape to a large extent. I have discovered that by vaporizing the metal and condensing the vapor in the manner hereinafter recited, it is practicable to obtain a product composed of particles of extreme fineness and uniformity and oxidized to only such an extent as not to interfere with the increased efficiency. The zinc dust of my invention is particularly efficient when used as a precipitant in the cyanide process of recovering precious metals.

The manufacture of zinc dust comprises, generally, vaporizing zinc and condensing the vapor. While it has been usual to vaporize the zinc in zinc ore, I prefer to use in this process zinc metal, slag, drosses, skimmings, residues or by-products of zinc metallurgical processes or any suitable zinc-bearing material. If the vapor therefrom is condensed in the air, the result is zinc oxide. If the vapor is condensed without air, the result is particles too large for efficient use. And either of these results may be observed in some of the particles obtained by following suggestions heretofore made. I have found that by giving proper attention to the supply of air in relation to the volume and tempera-

ture of the vapor, the difficulties are avoided and a superior product more expeditiously obtained.

To accomplish the result satisfactorily, it is desirable to supply to the vapor a carefully regulated supply of air, avoiding, on the one hand, complete exclusion of air from the condensing chamber (which would result in too large particles) and, on the other hand, an excessive amount of air in the condensing space or any part thereof (which would result in too much oxidation of the particles or some of them). This regulation of the supply of air may be accomplished by any means of admission which prevent any sudden inrush to any part of the condensing chamber. I have found that the apparatus hereinafter described affords one way of accomplishing it successfully and automatically.

It is preferable also to give attention to the heat of the vapor in connection with the regulated supply of air for limited oxidation. Because oxidation takes place more readily at high temperature, the supply of air should reach the vapor first at that point where it has parted with much of its latent heat. It is, accordingly, desirable to make use of a condensing chamber large enough to afford a cooling space and to admit the air at a point of comparatively low temperature therein.

In the accompanying drawing the apparatus described in my said application Serial No. 117,430, filed August 29, 1916, is shown as illustrating one convenient instrumentality which may be availed of for practising the process. The zinc-bearing material, preferably in the metallic form and with or without a quantity of carbon or other reducing agent, is placed in a retort 2, which is arranged in a furnace 3 so that it can be heated to the required temperature and in the apparatus which I have constructed, I employ oil as fuel. The neck of the retort extends through the furnace wall and makes a tight joint therewith and projects into a large neck 4 on the condensing chamber 5 and the joint between the furnace wall and the neck 4 is closed by clay seals 6. The neck 4 is made large in diameter so that the vapors passing from the retort will not be directed into contact therewith, since such contact has a tendency to form metallic zinc instead of zinc

dust. The chamber is preferably formed of metal and is in thermal contact with the air so that the heat therein may be dissipated. The chamber is preferably conical at its 5 lower end and is provided with a gate-controlled outlet 7, for the discharge of the dust. The chamber is provided with an aperture 8, preferably arranged on the side opposite the retort, which is covered with a bag 9 of suitable fabric, as for instance, woolen flannel. When vapor is discharged through the aperture, the bag becomes distended and when the pressure is relieved the bag collapses. As 10 the process is being carried on the bag pulsates continuously. The position of the aperture is preferably such that when the bag is removed, a stirring rod may be passed therethrough and into the retort.

When the process is practised by the use 20 of such apparatus a limited amount of air is presented to the vapor and contact of too much air with any part of the vapor (as might occur, for example, by permitting a sudden inrush of air to any part of the 25 condensing chamber on condensation) is avoided. This limited quantity of air is moreover presented to the vapor first at a point where the vapor has parted with some of its latent heat. The result is a dust, the 30 particles of which are extremely fine and uniform and oxidized to a limited extent, the oxidation being insufficient to interfere with the successful use of the product in the arts. By regulating the supply of air, the 35 percentage of oxidation may be accurately controlled to obtain a product best suited for the particular purpose in view.

The provision made for elasticity in the condensation chamber enables the vapor to 40 be properly separated from contact with too much oxygen during the period of condensation without creating such conditions of pressure or otherwise as result in condensation into comparatively large particles. 45 The maintaining of a proper equilibrium between the vapor, air and temperature at the time of condensation results in great uniformity of product and rapidity of production, as well as a more efficient article.

50 The standard method of determining the efficiency of zinc dust as a precipitant for gold or silver from cyanide solutions is the Sharwood method, set forth in the Journal of the Chemical, Metallurgical and Mining 55 Society of South Africa, vol. 12, No. 8 of page 332, February 1912, and reprinted in the Engineering and Mining Journal, vol. 93, No. 19, page 943, May 11, 1912. The Sharwood method is as follows:

"In testing for zinc efficiency a solution is prepared containing 8 grams of silver as potassium silver cyanide, 1.2 to 1.5 grams potassium cyanide, and .2 to .22 grams calcium oxide per liter. Emulsify .5 grams of the zinc dust with very little water, and add

250 cc. of the above solution with constant stirring. Continue stirring for ten minutes, and then stir violently every ten minutes for two hours. Filter rapidly and wash thoroughly, keeping precipitate in the 70 beaker. Dissolve in 10 cc. nitric acid (C. P.) and wash all precipitate off of filter with as little water as possible. Boil off fumes, cool, dilute to 250 cc., add ferric indicator, and titrate with standard solution 75 of a sulpho cyanide salt. Milligrams of silver found in this precipitate multiplied by the factor .0606 equals the precipitating efficiency when .5 grams of the zinc dust was used."

80 The zinc dust of my invention has an efficiency between 65% and 80% and the greater portion of the zinc dust made by my process has an approximate efficiency of about 78% by the Sharwood method, whereas the maximum efficiency of other zinc dusts formed by the condensation of zinc vapor is below 65% and averages about 55%.

85 I claim:

1. A process for manufacturing metal 90 dust, comprising vaporizing the metal and condensing the vapor in the presence of a limited regulated supply of oxygen.

2. A process for manufacturing metal 95 dust, comprising vaporizing the metal, supplying to the vapor a limited amount of air, first contacting with a comparatively cool portion of the vapor, and condensing the vapor in the presence of said supply of air.

100 3. A process for manufacturing metal dust, comprising vaporizing the metal, surrounding the vapor during the period of condensation with an elastic envelope adapted to expand and contract according to the volume of vapor and prevent unrestricted access of air to any portion of the vapor, and condensing the vapor within such envelope.

105 4. A process for manufacturing metal dust, comprising vaporizing the metal, maintaining said vapor out of contact with an unrestricted supply of air to any portion thereof, admitting to the vapor a restricted supply of air varyingly in proportion to the varying volume of the vapor, and condensing the vapor.

110 5. A process for manufacturing zinc dust, comprising vaporizing the zinc, condensing the vapor and oxidizing a portion thereof and controlling the oxidation.

115 6. A zinc dust composed of exceedingly fine particles substantially uniform in size and substantially uniformly oxidized, such as results from condensing zinc vapor in the presence of a limited supply of air without unrestricted access of air to any portion of the vapor during condensation.

120 7. A zinc dust resulting from the condensation of zinc vapor composed of substantially uniformly oxidized exceedingly fine 125

particles of zinc and having a precipitating efficiency above 65% as measured by the Sharwood method.

8. A zinc dust resulting from the condensation of zinc vapor composed of extremely fine particles of uniform structure, and having a precipitating efficiency above 70% as measured by the Sharwood method.

9. The process of manufacturing zinc dust, which consists in vaporizing the zinc, surrounding the vapor during the period of condensation with an envelop, supplying

to the envelop a limited amount of air first contacting with a comparatively cool portion of the vapor and condensing the vapor 15 in the presence of the supply of air, whereby zinc oxide and very fine zinc dust is formed.

In testimony whereof, I have hereunto set my hand at San Francisco, California, this 20 17th day of September, 1918.

MINTON H. NEWELL.

In presence of—  
H. G. PROST.